

UNITED STATES PATENT OFFICE

FREDERICK G. MOSES, OF NEW YORK, RAYMOND W. HESS, OF BUFFALO, AND ROBERT L. PERKINS, OF EAST AURORA, NEW YORK, ASSIGNEES TO THE BARRETT COMPANY, OF NEW YORK, N. Y., A CORPORATION OF NEW JERSEY

## SEPARATION OF MINERALS BY FLOTATION

No Drawing.

Application filed May 20, 1927. Serial No. 193,057.

This invention relates to the separation of minerals and the concentration of ores by flotation processes, and is particularly directed to such separation and concentration carried out with the utilization of certain organic sulfur bodies or compounds as flotation or mineral collecting agents.

According to the present invention, improved results can be obtained in the separation of minerals and the concentration of ores by carrying out the flotation operation with the addition to the ore or mineral pulp of a mercaptothiodiazole compound, particularly a mercapto-1:2:4-thiodiazole compound characterized by the formula



20 wherein R denotes a monovalent hydrocarbon radical which may contain substituents, and particularly denotes an aryl radical, more especially of the benzene series. The hydrogen atom of the mercapto group, i. e., the  
25 group, —SH, may be replaced by a metal to form a metal salt. It will be understood that said metallic salts are comprehended within the present invention. The flotation agents of the present invention may be prepared by  
30 methods described in the chemical literature.

In carrying out the flotation process, the flotation agent or adjuvant comprising the mercaptothiodiazole compound may be incorporated with the ore or the mineral pulp in any suitable manner and at any suitable time which will insure a satisfactory flotation operation. For example, it may be introduced in the free state or as a salt into the mill in which the ore is being ground, or it may be dissolved, suspended or dispersed in any suitable solvent or dispersing agent as, for example, in one or more of the usual flotation oils or oil mixtures, or in any suitable organic solvent or medium, or in water or in an alkali or alkaline reagent, and the resulting mixture incorporated with the ore or mineral pulp. While the agents of the present invention show marked action as flotation or mineral collecting agents in ore concentration, they in general exhibit insufficient

frothing qualities and are therefore usually employed to advantage in conjunction with any suitable or well-known frothing agent, e. g., pine oil, coal tar acids, terpineol, turpentine, etc. They may be also sometimes used to advantage in conjunction with other flotation agents. They may be used in the pure or purified state, and, in general, they may be also employed in the crude or impure state.

The process of the present invention can be carried out in any suitable apparatus, for example, those of the pneumatic type such as the Callow cell, or those where the air is incorporated with the pulp by agitation such as the Janney apparatus, or the like.

It is of advantage in some cases, as with certain copper ores, to subject the ore pulp to the action of an amount of alkali sufficient to give it an alkaline reaction before subjecting it to flotation with the aid of the flotation agents of the present invention. The alkali may be caustic alkali such as caustic soda, or an alkaline salt such as soda ash, or it may be calcium oxide or hydrate.

In the differential separation of various minerals, such as zinc blende from associated minerals, the presence of an alkali metal cyanide, or of copper sulfate or other salts, is sometimes advantageous.

The amount of flotation agent required to be used in the flotation process will vary, it depending partly on the character and composition of the ore, partly on the particular mercaptothiodiazole compound employed, and partly on other factors. In general, one-sixth to one-half pound of the flotation agent per ton of ore will be sufficient. Larger or smaller amounts of this, however, can be used. 85

This invention will be further illustrated by the following specific example, but it will be understood that the invention is not limited thereto. The parts are by weight. 90

Example: 500 parts of a copper sulfide ore (of the Inspiration Consolidated Copper Company) assaying 1.36 percent copper was ground in a ball mill with 250 parts water, 0.75 parts hydrated lime, and 0.0625 parts of 3-phenyl-5-mercapto-1:2:4-thiodiazole until practically all of it was sufficiently fine 100 95

to pass a 40-mesh screen. The ground pulp was diluted with sufficient water to give a mixture containing about 16 percent solids and subjected to flotation in a Janney mechanical apparatus. The mixture was agitated for 20 minutes during which time about 0.08 parts of pine oil was introduced. 67.3 parts of concentrate assaying 8.52 percent copper was obtained which is a recovery in the concentrate of 84.8 percent of the copper originally present in the heads. The tailings assayed 0.24 percent copper.

The present invention is of more or less general application to the treatment of various kinds of mineral substances, both natural and artificial, by flotation.

It will thus be noted that the present invention contemplates the utilization as flotation agents in the separation of minerals and the concentration of ores of mercaptothiodiazole compounds; that said flotation agents may be incorporated in or with the ore or mineral pulp at any suitable time or in any suitable manner; that they may be used in the free state or as salts or in admixture with one another or in solution, suspension or dispersion in any suitable solvent or medium; and that they may be used in conjunction with other flotation agents or with frothing agents, or with both.

It will be understood that the invention is not limited to the use of the particular agents or ingredients mentioned in the example and that other agents, particularly other flotation agents of the class specified, can be similarly used.

We claim:

1. In effecting the separation of minerals, the process which comprises incorporating 40 a mercaptothiodiazole compound with the mineral pulp, and subjecting the resulting mixture to a froth flotation operation.

2. In effecting the separation of minerals, the process which comprises incorporating 45 with the mineral pulp a mercaptothiodiazole compound corresponding in the free state with the following probable formula:



50 wherein R denotes a hydrocarbon radical which may contain substituents, and subjecting the resulting mixture to a froth flotation operation.

55 3. In effecting the separation of minerals, the process which comprises incorporating with the mineral pulp a mercaptothiodiazole compound corresponding in the free state with the following probable formula:



60 where R signifies an aryl radical or group, and subjecting the resulting mixture to a 65 froth flotation operation.

4. In effecting the separation of minerals, the process which comprises incorporating with the mineral pulp a mercaptothiodiazole compound corresponding in the free state with the probable formula:



70 wherein R denotes an aromatic hydrocarbon radical of the benzene series which may contain substituents, and subjecting the resulting mixture to a froth flotation operation.

75 5. In effecting the separation of minerals, the process which comprises incorporating with the mineral pulp 3-phenyl-5-mercaptop-1:2:4-thiodiazole, and subjecting the resulting mixture to a froth flotation operation.

80 6. In effecting the separation of minerals, the process which comprises incorporating with the mineral pulp a mercaptothiodiazole which in the free state embodies within its composition the following probable grouping:



85 and subjecting the resulting mixture to a froth flotation operation.

90 7. In effecting the concentration of a copper sulfide ore, the process which comprises subjecting a pulp of the ore to a froth flotation operation in the presence of a mercaptothiodiazole.

95 8. In effecting the concentration of a copper sulfide ore, the process which comprises subjecting a pulp of the ore to a froth flotation operation in the presence of a mercaptothiodiazole which in the free state embodies within its composition the following probable grouping:



100 9. In effecting the concentration of a copper sulfide ore, the process which comprises subjecting a pulp of the ore to a froth flotation operation in the presence of a mercaptothiodiazole having in the free state the following probable formula:



105 wherein R denotes an aryl group.

110 10. In effecting the concentration of a copper sulfide ore, the process which comprises subjecting a pulp of the ore to a froth flotation operation in the presence of a mercaptothiodiazole having in the free state the following probable formula:



115 In testimony whereof we affix our signatures.

FREDERICK G. MOSES.  
RAYMOND W. HESS.  
ROBERT L. PERKINS.

70

75

80

85

90

95

100

105

110

115

120

125

130